# EUROPEAN PATENT SPECIFICATION

(11) **EP 0 215 783 B1**
(45) Date of publication and mention of the grant of the patent: **17.07.1991**
(21) Application number: 85902289.9
(22) Date of filing: 16.04.1985
(51) Int. Cl.: B22C 3/00, B22C 9/02, B22C 9/10, B22C 9/12, B22D 17/20

(54) **COATING FOR MOLDS AND EXPENDABLE CORES**
BESCHICHTUNG FÜR GIESSFORMEN UND AUSDEHNBARE KERNE
REVETEMENT POUR DES MOULES ET POUR DES NOYAUX EXPANSIBLES

(43) Date of publication of application: 01.04.1987
(73) Proprietor: DOEHLER-JARVIS LIMITED PARTNERSHIP, Toledo, Ohio 43612 (US)
(72) Inventor: DYBALA, Charles, J., Toledo, OH 43611 (US); MACZKO, John, J., Port Clinton, OH 43623 (US)
(74) Representative: Gudel, Diether
(86) International application number: US8500675
(87) International publication number: WO8606012

(56) References cited:
- FR-A- 2 176 718
- FR-A- 2 466 293
- GB-A- 919 194
- US-A- 2 426 987
- US-A- 3 216 078
- US-A- 3 436 235
- US-A- 3 666 531
- US-A- 4 001 468
- US-A- 4 096 293
- US-A- 4 298 051
- US-A- 4 319 925
- US-A- 4 342 597
- US-A- 4 413 666
- PATENT ABSTRACTS OF JAPAN, vol. 6, no. 236 (M-173)[1114], 25th November 1982; & JP-A-57 134 236 (KUBOTA TEKKO K.K.) 19-08-1982
- PATENT ABSTRACTS OF JAPAN, vol. 6, no. 236 (M-173)[1114], 25th November 1982; & JP-A-57 134 237 (KUBOTA TEKKO K.K.) 19-08-1982

## Description

### Background of the Invention

The invention primarily relates to the art of die casting such metals as aluminum, zinc, magnesium, copper, iron and their alloys and to a solution to a long standing problem therein; i.e., the lack of a commercially feasible die casting technique to produce castings having undercut regions. More specifically, this invention relates to a coating composition useful on expendable die casting cores and particularly in pressurized die casting methods.

### Setting of the Invention

Traditional pressure die casting requires molds or dies which are able to withstand high temperatures and pressures. Ferrous materials are commonly used for such molds. Molds or cores of such materials for die castings having complex undercuts and reliefs are not possible since the cores for the undercut and relief cannot removed from the casting. To attain such complex undercuts and reliefs, sand cores which were expendable and fragile have been employed at pressures under 30 psia, i.e., gravity fed casting.

Sand cores have been employed for high pressure die castings and have been composed of sand mixed with a binding agent. The mixture is formed into the desired core shape and cured, bound together, by use of heat or chemical reaction. The cured core can then be used in the casting process.

The major problem with such expendable core in high pressure die casting methods has been the inability of the single binder system to meet four core requirements. These are a) good shake-out, b) good washout resistance, c) freedom from surface penetration, and d) strength.

Good shake-out is necessary to facilitate core removal from the casting.

Washout resistance is the ability of the core to withstand erosion from the high metal velocities that occur during injection of the molten metal. The washed out sand adversely affects tolerances on the finished part, since the sand may become embedded within the casting.

Surface penetration or hardness is caused by the combination of high heat and pressure which breaks down the core surface and permits the metal to penetrate between the sand grains thus causing a sand/metal mixture interface at the surface of the casting. This condition is detrimental to subsequent machining and machine tool life. Moreover, should the entrained sand become separated from the casting surface after component installation, damage to related parts, such as the lubrication system of an automobile engine, could result.

The strength of the core is determined mainly by the sand binder used. Therefore, suitable coating and compositions must be compatible with binders having desired strength.

### Prior Art

Although a wide variety of core and mold coatings have been developed for general foundry use, i.e., gravity fed casting, only a small number of coatings have been designed for the relatively harsh requirements connected with expendable high pressure die casting. Prior art coatings are illustrated by: US-A-4,096,293 discloses a core wash useful in pressurized die casting methods made of hydrocarbon solvent, fumaric resin, particulated calcium aluminate and a suspending agent. The composition comprises 5 to 90 wt% solvent, o,5 to 5 wt% resin, 5 to 80 wt% calcium aluminate and 0,1 to 2 wt% suspending agent. The fumaric resin is described as the reaction products of fumaric acid, gum rosin and pentaerythritol. The suspending agents are disclosed to include high molecular weight polymers, polyacrylates, colloidal silicas, clay, vegetable gums and amine-treated bentonite. Wetting agents are disclosed to include methyl alcohol, water and anionic and cationic surfactants.

The prior art is further illustrated by US-A-4,001,468 which discloses a wash coating useful for preventing core erosion. The composition of the coating includes an organic vehicle, suspending agent, refractory material and an organic polymer or copolymer. The organic vehicle is described as having a kauributanol value (ASTM D1133) of 36 or higher. The suspending agent is described as including clay, vegetable gums and amine-treated bentonite in ratio of suspending agent to vehicle of between 1:80 and 1:250. The refractory powder is described including graphite, coke, mica, silica, aluminium oxide, magnesium oxide, talc and zircon flour in a weight ratio of refractory to vehicle of between 1:2,5 and 1:3,5. The organic polymer or copolymer can be vinyl toluene butadiene polymer, styrene/butadiene copolymer, vinyl toluene/acrylate copolymer, styrene/acetylene copolymer, acrylate homopolymer, and styrene/butadiene copolymer in weight ratios of polymer/copolymer to vehicle between 1:50 and 1:200.

Disadvantages of said US-A include use of an organic binder which when heated releases an outgas which causes pores in the casting and lost strength. Further, these coatings are typically powdery and have reduced scratch resistance or hardness. Hardness is an indication of resistance to metal penetration or metal burning and erosion.

US-A-4,342,597 discloses to use a die casting sand core with a single coating consisting of an inorganic binder.

US-A-4,298,951 discloses to use a die casting sand core with an undercut where two identical coatings are provided consisting of organic bound coatings.

It is to be assumed that said both prior art die casting sand cores do not withstand high pressures.

### SUMMARY OF THE INVENTION

The invention in a first aspect consists in a strong die casting sand core comprising:
A) a base composed of a sand bound together by a binder;
B) a first coating comprising
   a) between about 30 and 80% by weight of an inorganic refractory material selected from graphite, mica, fused silica, aluminium oxide, magnesium oxide, carbon black and zircon flower, and
   b) between about 1% and 25% by weight of an inorganic binding agent selected from colloidal silica, clay and amine-treated bentonite,
   c) an aqueous liquid vehicle.
C) an additional top and second coating being provided and comprising:
   a) a refractory material selected from fused silica, zircon flower and aluminium oxide,
   b) an organic resin binding agent, and
   c) a liquid vehicle.

The invention in a second aspect consists in a method of coating a bonded sand core comprising sand bound together by a binder, the coating steps comprising:
A) first coating said cured sand core with a composition comprising:
   a) between about 30 to 80% by weight of an inorganic refractory material selected from the group consisting of graphite, mica, fused silica, aluminium oxide, magnesium oxide, carbon black and zircon flower,
   b) between about 1% and 25% by weight of an inorganic binding agent selected from the group consisting of colloidal silica, clay and amine-treated bentonite, and
   c) an aqueous liquid vehicle;
B) drying said first coating;
C) coating the dried coating with a second and top coating comprising:
   a) a refractory material selected from fused silica, zircon flower and aluminium oxide,
   b) an organic resin binding agent, and
   c) an organic liquid vehicle.

The invention in still another aspect consists in a method of forming a die casting having an undercut region comprising:
A) forming a die casting die having a casting surface that includes at least one expendable sand core that forms said undercut region, said sand core having good shake-out properties, good wash-out resistance, freedom from surface penetration, good shelf life and a high core strength to withstand pressures in excess of several thousand pounds per square inch;
B) forming said core comprising:
   a) a base composed of sand bound together by a binder,
   b) a first coating comprising:
      1) between about 30 to 80% by weight of an inorganic refractory material selected from graphite, mica, fused silica, aluminium oxide, magnesium oxide, carbon black and zircon flower,
      2) and between about 1% and 25% by weight of an inorganic binding agent selected from colloidal silica, clay and amine-treated bentonite,
      3) an aqueous liquid vehicle;
C) an additional top and second coating comprising:
   1) a refractory material selected from fused silica, zircon flower and aluminium oxide,
   2) an organic resin binding agent,
   3) a liquid vehicle;
D) placing said formed core in said die casting die;
E) injecting molten metal into said die casting die;
F) permitting said injected molten metal to solidify to form said die casting having said undercut region;
G) removing said die casting from said die; and
H) separating said expendable core from said undercut region within said die casting.

The essential features of the invention, therefore, are a core and first mold wash composition comprising:
a) particulate refractory material,
b) inorganic binding agent and
c) liquid vehicle

and a second and different composition top wash coating comprising:
a) refractory material,
b) binding agent, and
c) liquid vehicle.

In said second aspect, this invention comprises a method of treating a foundry core or mold by coating the surface of the sand core or mold with a wash of the foregoing composition.

In said third aspect, this invention comprises a mold and expendable core coated with the foregoing composition.

### Detailed Description of the Invention

The first core wash coating of this invention comprises particulate refractory material, an inorganic binding agent and a liquid vehicle. This coating is suitable for use on sand cores and molds which are useful in die casting as well as in gravity fed casting. This invention meets the four core requirements through the use of a core system having a coating/binder system that enhances shakeouts, washout resistance and surface penetration resistance. The wash coatings can also include such secondary components such as fungicides, wetting agents and defoaming agents.

The wash coatings are useful on uncoated inorganic and organic sand and binder agent cores which provide good shakeout characteristics but fall to have suitable washout surface penetration resistance and effect in strength. Preferably, the binder agent of the core is a organic resin. More preferably, the agent is an acid curable organic resin and oxidizing agent which is cured by exposure to sulfur dioxide.

Suitable refractory materials for this invention should not react with the binder agent and are graphite, mica, fused silica, aluminium oxide, magnesium oxide, carbon black and zircon flour.

The refractory material is selected from the group consisting of fused silica, zircon flour and aluminium oxide. Preferably, refractory material is fused silica. The refractory material should preferably have a particle size ranging from about 1 to 100 microns. Fused silica having a particle size within the range of about 1 and about 45 microns is most preferred. Preferably, the fused silica is wet milled.

The first wash coating comprises an inorganic binding agent such as colloidal silica, clay, or amine-treated bentonite or a combination thereof. Preferably, the suspending agent is selected from a group consisting of colloidal silicas, clays and bentonite. More preferably, the agent is colloidal silica.

The liquid vehicle may be either aqueous or organic. Selection of the vehicle is usually based on the type of binder used to bind the sand of the foundry core and mold. If the core binder is aqueous, the vehicle for the coating should preferably be organic. If the core binder is organic, the vehicle for the coating should preferably be aqueous.

Preferably the composition of the core wash should range from about 30 to 80 wt % refractory material, from about 1 to about 25 wt % binder agent and from about 20 to 70 wt % liquid vehicle. The more preferred composition ranges from about 50 to 70 wt % refractory material, about 5 to 12 wt % binder agent and about 25 to about 40 wt % liquid vehicle. The most preferred composition is about 62 wt % refractory material, about 8 wt % binder agent and about 30 wt % liquid vehicle.

The wash coating should preferably form a coating on the sand core having a thickness ranging from about 250 to about 5000 microns. The preferred range of thickness is between 1000 and about 3000 microns.

To prepare an expendable core of the invention, sand and binding agent are mixed and air blown or hand-packed into a core box having the desired shape of the core. The core is cured by heating or passing a suitable gas through the core box. The core is removed from the box as a solid mass.

The coating may then be applied to the core by conventional techniques such as dipping or spraying the core. The coating may be applied as single or multiple coats. The core and coating are then allowed to dry.

The coating of this invention is covered with a top wash coating containing a refractory material, binding agent, preferably suspending agent and a liquid vehicle. The second coating improves protection of the core and facilitation of core removal from the casting.

The refractory material of the top wash coating is selected from the group consisting of fused silica, zircon flour and aluminium oxide. Preferably, the material is zircon flour.

The suspending agent of the top wash coating may be selected from a group consisting of high molecular weight polymers and copolymers, silicas, vegetable gums, clays and combination thereof. Preferably, the suspending agent of the top wash is selected from a group consisting of colloidal silicas, clays, and bentonite. More preferably, the agent is colloidal silica.

The binding agent of the top wash coating is organic and may be selected from suitable agents such as polymer resins.

The liquid vehicle of the top wash is organic. Selection of the vehicle is usually based on the type of binder used to bind the sand of the foundry core and mold as well as the first coating. It the binder is aqueous, the vehicle for the coating should preferably be organic. More preferably, the top coating comprises zirconium silicate, resin binder and isopropyl alcohol. The top wash coating should preferably form a cured coating on the sand core having a thickness ranging from about 100 to about 2000 microns and the preferred range is from about 250 to 1000 microns.

The second wash coating may be applied as single or multiple coats.

### Example 1

An expendable sand core was formed of 97.90 wt % silica foundry sand (AFS Fineness No. 65), 1.47 % furane and 0.59 wt % methyl ethyl ketone peroxide, and 0.04 wt % silane. The core was treated with sulfur dioxide for two seconds at ambient temperature and pressure.

A core wash composition was prepared containing various levels of fused silica, colloidal silica and water, the fused silica particles ranging in size from 1 to 45 microns. The composition was milled by introducing porcelain balls into a container of the composition and rotating the container for two to three hours to break up large agglomerated particles. The milled composition was poured through a cloth paint strainer. The specific gravity of the composition was then checked and adjusted by addition of fused silica or colloidal silica slurry until the Baume reading fell within the range of 56 and 62. Approximately 10% by volume of methanol was added. An additional amount of kaolin was added to the composition which was then stirred for a minimum of one hour. The composition was then allowed to stand for 24 hours.

The coated cured core was used to produce a complex aluminum alloy die casting having an undercut region. The core was removed from the casting using conventional mechanical shakeout techniques. The core and casting were tested for shakeout, washout and penetration and rated for each characteristic.

### Example 2

A cured coated core of Example 1 was dipped in the core wash composition for approixmately ten seconds, removed and drained. The coat was allowed to dry. The dry coated core was dipped again in the core wash composition for about five seconds, drained and dryed in a circulating air oven at 175°F for at least three minutes. A casting was made using the core and both were rated as in Example 1.

### Example 3

An uncoated expendable core was prepared as in Example 1, a casting prepared therefrom and the core and casting were tested and rated as in Example 1.

### Example 4

A coated expendable core was prepared as in Example 1. This core was cooled for at least two minutes and dipped in a top coating composition containing zirconium silicate, a resin binder, and isopropyl alcohol (Arcolite #412, Atlantic Richfield Co.) for two to three seconds. The core was drained and allowed to air dry for 30 minutes. A casting was made using the core.

The double-coated core and the casting were rated for shakeout, washout and penetration.

### Example 5

An uncoated expendable core as prepared as in Example 3 was dipped in the zirconium silicate/resin binder coating composition of Example 4 and allowed to dry. A casting was made of the coated core and casting were rated.

## Claims

1. A strong die casting sand core comprising:
A) a base composed of a sand bound together by a binder;
B) a first coating comprising
a) between about 30 and 80% by weight of an inorganic refractory material selected from graphite, mica, fused silica, aluminium oxide, magnesium oxide, carbon black and zircon flower, and
b) between about 1% and 25% by weight of an inorganic binding agent selected from colloidal silica, clay and amine-treated bentonite,
c) an aqueous liquid vehicle.
C) an additional top and second coating being provided and comprising:
a) a refractory material selected from fused silica, zircon flower and aluminium oxide,
b) an organic resin binding agent, and
c) a liquid vehicle.

2. A strong die casting sand core according to claim 1, wherein said top coating comprises a suspending agent selected from colloidal silica, clay and vegetable gums.

3. A sand core according to claim 1 or 2, wherein said base binder comprises an organic resin.

4. A sand core according to any of claims 1 to 3, wherein said first coating is between 250 and 5000 microns thick.

5. A sand core according to any of claims 1 - 4, wherein said second coating is between about 100 and 2000 microns thick.

6. A high pressure die casting made with a core according to any of claims 1 - 5.

7. A method of coating a bonded sand core comprising sand bound together by a binder, the coating steps comprising:
A) first coating said cured sand core with a composition comprising:
a) between about 30 to 80% by weight of an inorganic refractory material selected from the group consisting of graphite, mica, fused silica, aluminium oxide, magnesium oxide, carbon black and zircon flower,
b) between about 1% and 25% by weight of an inorganic binding agent selected from the group consisting of colloidal silica, clay and amine-treated bentonite, and
c) an aqueous liquid vehicle;
B) drying said first coating;
C) coating the dried coating with a second and top coating comprising:
a) a refractory material selected from fused silica, zircon flower and aluminium oxide,
b) an organic resin binding agent, and
c) an organic liquid vehicle.

8. A method according to claim 7 wherein said top coating comprises a suspending agent selected from colloidal silica, clay, vegetable gums and bentonite.

9. A method of coating according to claim 7 or 8 wherein said base binder comprises an organic resin.

10. A method of coating according to any of claims 7 - 9 wherein said first coating is between about 250 and 5000 microns thick.

11. A method of coating according to any of claims 7 - 10 wherein said second coating is between about 100 and 2000 thick.

12. A method of forming a die casting having an undercut region comprising:
A) forming a die casting die having a casting surface that includes at least one expendable sand core that forms said undercut region, said sand core having good shake-out properties, good wash-out resistance, freedom from surface penetration, good shelf life and a high core strength to withstand pressures in excess of several thousand pounds per square inch;
B) forming said core comprising:
a) a base composed of sand bound together by a binder,
b) a first coating comprising:
1) between about 30 & 80% by weight of an inorganic refractory material selected from graphite, mica, fused silica, aluminium oxide, magnesium oxide, carbon black and zircon flower, and
2) between about 1% and 25% by weight of an inorganic binding agent selected from colloidal silica, clay and amine-treated bentonite,
3) an aqueous liquid vehicle;
C) an additional top and second coating comprising:
1) a refractory material selected from fused silica, zircon flower and aluminium oxide,
2) an organic resin binding agent,
3) a liquid vehicle;
D) placing said formed core in said die casting die;
E) injecting molten material into said die casting die;
F) permitting said injected molten material to solidify to form said die casting having said undercut region;
G) removing said die casting from said die; and
H) separating said expendable core from said undercut region within said die casting.

13. A method according to claim 12 wherein said top coating comprises a suspending agent selected from colloidal silica, clay, vegetable gums and bentonite.

## Revendications

1. Noyau de sable pour coulage sous pression résistant comprenant :
A) une base composée d'un sable lié par un liant ;
B) un premier enduit comprenant
**a)** entre environ 30 et 80% en poids d'une matière réfractaire inorganique choisie parmi le graphite, le mica, la silice fondue, l'oxyde d'aluminium, l'oxyde de magnésium, le noir de fumée et la fleur de zircon, et
**b)** entre environ 1% et 25% en poids d'un agent liant inorganique choisi parmi la silice colloïdale, l'argile et la bentonite traitée avec une amine,
**c)** un véhicule liquide aqueux.
C) un enduit supérieur et second additionnel et supérieur étant fourni et comprenant :
**a)** une matière réfractaire choisie parmi la silice fondue, la fleur de zircon et l'oxyde d'aluminium,
**b)** un agent liant de résine organique, et
**c)** un véhicule liquide.

2. Noyau de sable pour coulage sous pression résistant selon la revendication 1, dans lequel ledit enduit supérieur comprend un agent de suspension choisi parmi la silice colloïdale, l'argile et les gommes végétales.

3. Noyau de sable selon la revendication 1 ou 2, dans lequel ledit liant de base comprend une résine organique.

4. Noyau de sable selon l'une quelconque des revendications 1 à 3, dans lequel ledit premier enduit a une épaisseur comprise entre 250 et 5000 microns.

5. Noyau de sable selon l'une quelconque des revendications 1 à 4, dans lequel ledit second enduit a une épaisseur comprise entre environ 100 et 2000 microns.

6. Coulage sous haute pression fait avec un noyau selon l'une quelconque des revendications 1 à 5.

7. Procédé de revêtement d'un noyau de sable lié comprenant du sable retenu assemblé par un liant, les étapes de revêtement comprenant :
A) tout d'abord le revêtement dudit noyau de sable durci avec une composition comprenant :
**a)** entre environ 30 et 80% en poids d'une matière réfractaire inorganique choisie dans le groupe constitué par le graphite, le mica, la silice fondue, l'oxyde d'aluminium, l'oxyde de magnésium, le noir de fumée et la fleur de zircon;
**b)** entre environ 1% et 25% en poids d'un agent liant inorganique choisi dans le groupe constitué par la silice colloïdale, l'argile et la bentonite traitée avec une amine, et
**c)** un véhicule liquide aqueux ;
B) le séchage dudit premier enduit ;
C) l'enduction de l'enduit séché avec un enduit second et supérieur comprenant :
**a)** une matière réfractaire choisie parmi la silice, la fleur de zircon et l'oxyde d'aluminium,
**b)** un agent liant de résine organique, et
**c)** un véhicule liquide organique.

8. Procédé selon la revendication 7, dans lequel ledit enduit supérieur comprend un agent de suspension choisi parmi la silice colloïdale, l'argile, les gommes végétales et la bentonite.

9. Procédé de revêtement selon la revendication 7 ou 8, dans lequel ledit liant de base comprend une résine organique.

10. Procédé de revêtement selon l'une des revendications 7 à 9, dans lequel ledit premier enduit a une épaisseur comprise entre environ 250 et 5000 microns.

11. Procédé de revêtement selon l'une quelconque des revendications 7 à 10, dans lequel ledit second enduit a une épaisseur comprise entre environ 100 et 2000.

12. Procédé de formation d'un coulage sous pression ayant une région d'évidement dans lequel :
A) on forme un moule pour coulage sous pression ayant une surface de coulée qui inclut au moins un noyau de sable expansible qui forme ladite région à coupe inférieure à la cote, ledit noyau de sable ayant de bonnes propriétés de décochage , une bonne résistance au lavage, une bonne résistance à la pénétration à la surface, une bonne durée de conservation et une résistance élevée du noyau afin de résister à des pressions dépassant plusieurs dizaines de MPa ;
B) On forme ledit noyau comprenant :
**a)** une base composée de sable lié par un liant ;
**b)** un premier enduit comprenant :
1) entre environ 30 et 80% en poids d'une matière réfractaire inorganique choisie parmi le graphite, le mica, la silice fondue, l'oxyde d'aluminium, l'oxyde de magnésium, le noir de fumée et la fleur de zircon, et
2) entre environ 1% et environ 25% en poids d'un agent liant inorganique choisi parmi la silice colloïdale, l'argile et la bentonite traitée avec une amine,
3) un véhicule liquide aqueux ;
C) un enduit supérieur et second additionnel comprenant :
1) une matière réfractaire choisie parmi la silice fondue, la fleur de zircon et l'oxyde d'aluminium,
2) un agent liant de résine organique,
3) un véhicule liquide ;
D) On place ledit noyau formé dans ledit moule de coulage sous pression ;
E) On injecte la matière fondue dans ledit moule de coulage sous pression ;
F) On permet à ladite matière fondue injectée de se solidifier pour former ledit coulage sous pression ayant ladite région d'évidement ;
G) On enlève ledit moulage sous pression dudit moule ; et
H) On sépare ledit noyau expansible de ladite région à évidement dans ledit coulage sous pression.

13. Procédé selon la revendication 12, dans lequel ledit enduit supérieur comprend un agent de suspension choisi parmi la silice colloïdale, l'argile, les gommes végétales et la bentonite.

## Patentansprüche

1. Belastbarer Sandkern für eine Gießform mit
A) einem Grundmaterial aus Sand, der mit einem Bindemittel gebunden ist,
B) einer ersten Beschichtung mit
a) etwa 30 bis 80 Gew.% eines anorganischen Auskleidungsmaterials, ausgewählt aus Graphit, Glimmer, geschmolzenem Sikika, Aluminiumoxid, Magnesiumoxid, Ruß und Zirkonblume, und
b) etwa 1 bis 25 Gew.% eines anorganischen Bindemittels, ausgewählt aus kolloidalem Silika, Ton und amino-behandeltem Bentonit,
c) einem flüssigen Träger
und mit
C) einer zusatzlichen oberen und zweiten Beschichtung mit
a) einem Auskleidungsmaterial, ausgewählt aus geschmolzenem Silika, Zirkonblume und Aluminiumoxid,
b) einem Bindemittel aus organischem Harz und mit
c) einem flüssigen Träger.

2. Sandkern nach Anspruch 1,
**dadurch gekennzeichnet,**
daß die obere Beschichtung ein suspendiertes Mittel aus kolloidalem Silika, Ton oder pflanzlichen Harzen aufweist.

3. Sandkern nach Anspruch 1 oder 2,
**dadurch gekennzeichnet,**
daß das Bindemittel ein organisches Harz aufweist.

4. Sandkern nach einem der Ansprüche 1 bis 3,
**dadurch gekennzeichnet,**
daß die erste Beschichtung zwischen 250 und 5.000 Mikron dick ist.

5. Sandkern nach einem der Ansprüche 1 bis 4,
**dadurch gekennzeichnet,**
daß die zweite Beschichtung zwischen etwa 100 und 2.000 Mikron dick ist.

6. Hochdruck-Gießform, hergestellt mit einem Kern nach einem der Ansprüche 1 bis 5.

7. Verfahren zum Beschichten eines gebundenen Sandkerns, der mit einem Bindemittel gebundenen Sand enthält,
**dadurch gekennzeichnet,**
daß
A) der gehärtete Sandkern zunächst mit einer Zusammensetzung beschichtet wird, die folgende Bestandteile aufweist:
a) etwa 30 bis 80 Gew.% eines anorganischen Auskleidungsmaterials, ausgewählt aus Graphit, Glimmer, geschmolzenem Silika, Aluminiumoxid, Magnesiumoxid, Ruß und Zirkonblume,
b) etwa 1 bis 25 Gew.% eines anorganischen Bindemittels, ausgewählt aus kolloidalem Silika, Ton und amino-behandeltem Bentonit, und
c) einem flüssigen Träger,
B) daß die erste Beschichtung getrocknet wird,
C) daß die getrockenete Beschichtung mit einer zweiten und oberen Beschichtung beschichtet wird, die folgende Bestandteile aufweist:
a) ein Auskleidungsmaterial, ausgewählt aus geschmolzenem Silika, Zirkonblume und Aluminiumoxid,
b) ein Bindemittel aus organischem Harz und
c) einen flüssigen Träger.

8. Verfahren nach Anspruch 7,
**dadurch gekennzeichnet,**
daß die obere Beschichtung ein suspendiertes Mittel aufweist, das aus kolloidalem Silika, Tonerde, pflanzlichen Harzen oder Bentonit besteht.

9. Verfahren nach Anspruch 7 oder 8,
**dadurch gekennzeichnet,**
daß das Grundbindemittel ein organisches Harz aufweist.

10. Verfahren nach einem der Ansprüche 7 bis 9,
**dadurch gekennzeichnet,**
daß die erste Beschichtung etwa zwischen 250 und 5.000 Mikron dick ist.

11. Verfahren nach einem der Ansprüche 7 bis 10,
**dadurch gekennzeichnet,**
daß die zweite Beschichtung etwa zwischen 100 und 2.000 Mikron dick ist.

12. Verfahren zum Formen einer Gießform mit einer Hinterschneidung,
**dadurch gekennzeichnet,**
daß
A) eine Gießform mit einer Gießfläche mit wenigstens einem ausdehnbaren Sandkern geformt wird, der die Hinterschneidung ausbildet, wobei der Sandkern gute Ausgleichseigenschaften hat, einen guten Auswaschwiderstand, frei ist von Eindringen in die Oberfläche, eine gute Lebensdauer hat und eine hohe Kernfestigkeit derart, daß der Kern Drücken über mehrere tausend Pfund pro Quadratzoll widerstehen kann,
B) daß der Sandkern geformt wird, der folgende Materialien aufweist:
a) ein Grundmaterial aus Sand, der mit einem Bindemittel gebunden ist,
b) eine erste Beschichtung mit
1) etwa 30 bis 80 Gew.% eines anorganischen Auskleidungsmaterials, ausgewählt aus Graphit, Glimmer, geschmolzenem Sikika, Aluminiumoxid, Magnesiumoxid, Ruß und Zirkonblume, und
2) etwa 1 bis 25 Gew.% eines anorganischen Bindemittels, ausgewählt aus kolloidalem Silika, Ton und amino-behandeltem Bentonit,
3) einem flüssigen Träger,
C) eine zusätzliche obere und zweite Beschichtung mit
1) einem Auskleidungsmaterial, ausgewählt aus geschmolzenem Silika, Zirkonblume und Aluminiumoxid,
2) einem Bindemittel aus organischem Harz und mit
3) einem flüssigen Träger,
D) daß der geformte Kern in die Gießform eingesetzt wird,
E) daß geschmolzenes Material in die Gießform injiziert wird,
F) daß das injizierte, geschmolzene Material zur Formung des Gußstücks mit der Hinterschneidung verfestigt wird,
G) daß das Gußstück aus der Form entfernt wird und
H) daß der ausdehnbare Kern aus der Hinterschneidung in dem Gußstück abgetrennt wird.

13. Verfahren nach Anspruch 12,
**dadurch gekennzeichnet,**
daß die obere Beschichtung ein suspendiertes Mittel aus kolloidalem Silika, Tonerde, pflanzlichen Harzen oder Bentonit aufweist.
